

June 26, 1945.

M. J. ZUNICK

2,379,397

ANODE STRUCTURE

Filed Nov. 16, 1942



INVENTOR:  
Michael J. Zurick,  
BY:

Spencer, Marshall, Johnston & Cook,  
Attn:

## UNITED STATES PATENT OFFICE

2,379,397

## ANODE STRUCTURE

Michael J. Zunick, Columbus, Ohio, assignor to  
General Electric X-Ray Corporation, Chicago,  
Ill., a corporation of New York

Application November 16, 1942, Serial No. 465,715

15 Claims. (Cl. 250—149)

My invention relates in general to electronics and has more particular reference to an improved electrode construction particularly well suited for anodes of X-ray generators.

An X-ray generator comprises an electron emitting cathode and an anode at which X-rays are generated by impingement, upon a suitable target at the anode, of electrons emitted by the cathode. Among materials commonly used for anode targets are tungsten, nickel, copper, cobalt, iron, chromium, molybdenum, and other metals. Electron impingement on the target surface of the anode during operation of the tube results in grain growth in the target material at the target surface due to heat, liberated in the anode through electron impingement thereon. Such grain growth results in deformation or curling of the anode at the target surface and consequent reduction in the X-ray output of the generator; and an important object of the present invention is to minimize such target deformation or curling through the provision of an improved anode structure presenting the anode material at the target surface in dense condition having a grain structure and other characteristics particularly well adapted to resist target deformation or curling.

Another object is to minimize target deterioration by employing a target of pure metal; a further object being to utilize pure electrolytic copper.

Another important object is to provide an anode for an X-ray generator having a target surface comprising material in which the grain structure extends in a direction intersecting the plane of the target surface preferably at right angles; a further object being to utilize as an X-ray anode target a button in which the metallic grain structure extends in a direction normal to the target face of the button; a still further object being to form target buttons by first rolling a bar of suitable metallic target material longitudinally to impart a grain structure extending lengthwise of the bar and then cutting discs from the bar to provide buttons in which the grain structure comprises grains having ends extending at the cut face of the button.

The foregoing and numerous other important objects, advantages, and inherent functions of the invention will be fully understood from the following description, which, taken in connection with the accompanying drawing, discloses a preferred embodiment of the invention.

Referring to the drawing:

Figure 1 is a sectional view taken through an

X-ray generator fitted with an anode embodying the present invention;

Figure 2 is a sectional view taken substantially along the line 2—2 in Figure 1;

Figure 3 is an enlarged sectional view taken substantially along the line 3—3 in Figure 2; and

Figure 4 is a section view similar to Figure 3 showing a modified anode structure embodying the invention.

To illustrate the invention the drawing shows an X-ray generator 11 comprising a sealed envelope 13 containing an anode 15 and a cathode 17 embodying an electron emitting filament 19, the cathode and anode being mounted in coaxial spaced and facing relationship within the envelope 13. Suitable conductors for energizing the filament 19 and for applying operating potential between the filament and the anode from an electrical power source outwardly of the envelope, of course, are provided.

While the invention is not necessarily limited to any particular type or form of generator, the X-ray generator 11, as shown in Figure 1, comprises a generator of the short particularly well suited for producing X-rays for the analysis of materials by X-ray diffraction. To this end the surface of the anode facing the electron emitting element 19 forms a target surface 21, and the generator operates to produce X-rays at said target surface as a result of the impingement, on said surface, of electrons emitted at the filament 19 when electrically energized, said emitted electrons being impelled toward and caused to impinge upon the target surface 21 under the influence of generator operating electrical potential applied between the filament and the anode. The target surface 21 may, of course, comprise any suitable metallic material, such as tungsten, molybdenum, copper, nickel, cobalt, iron, chromium or other preferred target material.

X-rays generated as a result of electron impingement on the target surface 21 pass outwardly of the envelope through transmitting windows 23 formed in the envelope walls opposite the anode target. If desired, the envelope of the generator may be enclosed in a casing, or a sleeve 25 of X-ray opaque material, and may be assembled around the X-ray transmitting portions 50 of the envelope and provided with openings 27 in line with the windows 23 for the purpose of blocking exit of X-rays from the tube except at said openings 27.

When an X-ray generator is in operation for production of X-rays at the target 21, a consid-

erable amount of heat is developed at the target surface as a result of electron impingement, such heat being dissipated through the body of the anode and thence outwardly of the envelope. The temperature at the target surface of the anode, however, may be of the order of the melting temperature of the target material, it being usual, in the interests of operating efficiency, to operate the generator so that its anode at the target surface functions at a temperature just short of the softening temperature of the anode material. When operated at such temperature there is a tendency for grain growth to occur in the anode material, such growth being evidenced by the bulging or curling of the anode material at the target surface and the consequent deformation of said surface from a desirable flat condition. Such deformation or curl, to some extent, impairs the production of X-rays at the target of the device.

According to the present invention, the tendency of the target surface to become raised or curled in service is minimized by providing a target comprising substantially pure metal. To this end, where the target is formed of copper, pure electrolytic copper is preferably employed as the target material. Likewise, where other target material, such as tungsten, chromium, nickel, cobalt, iron, molybdenum or other metal is employed, appreciable improvement is obtained in the ability of the target to resist deterioration in service, when the target material is applied and maintained in substantially pure form.

Target deformation and curling in service also is minimized by using compact, dense metal having a uniform grain structure characterized, preferably, in that the grains of the material extend vertically with respect to the target surface of the anode. Electrons impinging on such a surface strike the ends of the crystals of material forming the anode target, which, because of the compact parallel grain structure, tends to avoid grain growth. The structure of material having parallel grain arrangement, with the grain ends presented at the target surface, may conveniently be designated by the term "end grain."

While the entire anode may be formed of material having the desired grain structure, including grains ending or terminating at the target surface, it is not necessary to make the entire anode of the relatively expensive end grain material, and it is preferable to form the body 29 of the anode in any suitable or convenient manner, as by forming the same as a casting, preferably comprising vacuum melting copper.

The body of the anode, however, is formed with a pocket 31 in the surface thereof which faces the cathode and a target button 33 is fixed in said pocket, as by soldering the same in place. The button 33, in the illustrated embodiment, comprises a suitable metallic target material, such as pure electrolytic copper, or other metallic target material, in which the grains extend in a direction normal to the target surface 21 of the button. Such granular structure may be accomplished by rolling or otherwise working a bar of the selected target material in order to accomplish the desired parallel grain structure in a direction longitudinally of the bar, and then cutting the bar in sections at right angles to the grain direction in order to provide the target button 33, having the so-called "end grain" structure.

The button 33 may be secured in the pocket 31 by soldering the same in place, as with eutectic

silver solder 35, comprising the alloy of silver with twenty-eight per cent. of copper. The employment of an anode embodying end grain target material materially improves the curl-resisting ability of the target. At the same time, it is equally important, if not more important, to employ a target material comprising pure metal. In making a copper target, pure electrolytic copper should be used as the target material. Commercial vacuum melted copper of the sort ordinarily employed in X-ray tube anodes is appreciably contaminated with foreign material and shows a very definite tendency to blister or curl when used as a target material, even if treated to provide vertical grain structure. Pure electrolytic copper, however, even in the absence of the desirable end grain arrangement, provides a satisfactory substantially non-bulging target, the same being true where other target materials are used in substantially pure condition for target purposes. The end grain arrangement, however, is of appreciable value in producing satisfactory anodes and consequently the same forms a valuable phase of the present invention.

When in operation at high temperature there is a tendency for the solder 35 to flow along and between the parallel grains of the button 33, and solder may, in this way undesirably reach the face of the target.

In order to exclude the possibility of solder flow along and between the crystals of a soldered end grain target button, the same may be directly united with a backing disc 37 of like material in which the grains extend crosswise of the disc, as shown in Figure 4. The composite backed button thus produced may be soldered in the pocket 31 without any possibility of solder flow therethrough to the face of the target.

X-ray tube anodes made in accordance with the teachings of the present invention are characterized in that they are substantially immune to target surface deformation in service.

It is thought that the invention and its numerous attendant advantages will be fully understood from the foregoing description, and it is obvious that numerous changes may be made in the form, construction and arrangement of the several parts without departing from the spirit or scope of the invention, or sacrificing any of its attendant advantages, the form herein disclosed being a preferred embodiment for the purpose of illustrating the invention.

The invention is hereby claimed as follows:

1. An anode structure comprising a body of pure electrolytic copper forming a target surface, said body having an internal grain structure normal to the target surface.
2. An anode structure comprising a body of metal forming a target surface, said body having an internal grain structure normal to the target surface.
3. An anode structure comprising a body of metal forming a target surface, said body being in substantially pure condition without contamination and having an internal grain structure substantially normal to the target surface.
4. An anode structure comprising a copper base having a pocket and a body of metal forming a target button secured in said pocket, said button forming a target surface and having an internal grain structure normal to the target surface.
5. An anode structure comprising a base of vacuum cast copper formed with a pocket and a metallic target button secured in said pocket,

said button providing a target surface and having an end grain structure at said surface.

6. An anode structure comprising a copper base having a pocket and a body of pure electrolytic copper forming a target button secured in said pocket, said button forming a target surface and having an internal grain structure normal to the target surface.

7. An anode structure comprising a base of vacuum cast copper formed with a pocket and a target button of pure electrolytic copper secured in said pocket, said button forming a target surface and having an internal grain structure normal to the target surface.

8. An anode structure comprising a base having a pocket, a metal target button having end grain structure secured in the pocket, and a backing disc of metal in the pocket behind said target button.

9. An anode structure comprising a base having a pocket, a metal target button having end grain structure secured in the pocket, and a backing disc of metal in the pocket behind said target button, said backing disc having cross grain structure.

10. An anode structure comprising a metallic base having a pocket, a metal target button having end grain structure in said pocket, and a backing disc of metal in the pocket behind said target button and directly bonded to said target button, said backing disc having internal cross grain structure and being soldered in place in the pocket whereby to prevent contamination of the target button by the solder.

11. An anode structure comprising a base having a pocket, and a target button secured in said

5 pocket and having a target surface, said target button comprising metal having an internal grain structure substantially normal to the target surface.

12. An anode structure comprising a copper base having a pocket, and a target button secured in said pocket and providing a target surface, said target button comprising metal in substantially pure condition without contamination and having an internal grain structure substantially normal to the target surface.

13. An anode structure comprising a base of vacuum cast copper formed with a pocket, and a target button secured in said pocket and providing a target surface, said target button comprising metal in substantially pure condition without contamination and having an end grain structure at said surface.

14. An anode structure comprising a base having a pocket, a target button secured in said pocket and providing a target surface, said button comprising metal in substantially pure condition without contamination and having an end grain structure at said surface, and a backing disc of metal in the pocket behind said target button.

15. An anode structure comprising a base having a pocket, a target button secured in said pocket and providing a target surface, said button comprising metal in substantially pure condition without contamination and having an end grain structure at said surface, and a backing disc of metal in the pocket behind said target button, said backing disc having cross grain structure.

MICHAEL J. ZUNICK.